

April 11, 1939.

J. EGGERT ET AL

2,153,617

MANUFACTURE OF COLORED PHOTOGRAPHIC PICTURES

Filed June 18, 1936



John Eggert  
Bruno Wendt  
Inventors

By their Attorneys *John*

## UNITED STATES PATENT OFFICE

2,153,617

MANUFACTURE OF COLORED PHOTO-  
GRAPHIC PICTURES

John Eggert, Leipzig-Gohlis, and Bruno Wendt,  
Dessau, Germany, assignors, by mesne assign-  
ments, to Agfa Ansco Corporation, Binghamton,  
N. Y., a corporation of New York

Application June 18, 1936, Serial No. 85,848  
In Germany June 22, 1935

2 Claims. (Cl. 95—2)

Our present invention relates to the manufac-  
ture of colored photographic pictures.

One of its objects is to provide a process for  
producing improved colored photographic pic-  
tures. Another object is the provision of a ma-  
terial on which the improved pictures are pro-  
duced. Further objects will be seen from the  
detailed specification following hereinafter.

The single figure of the accompanying drawing  
10 shows a film for use in accordance with the in-  
vention.

The manufacture and application of colored  
filter layers which contain dyestuffs stable to the  
developing and fixing baths is known.

15 The use of such colored layers in a multi-layer  
material produces pictures in natural colors only  
with great difficulty when the known methods are  
applied. For producing colored cinematograph  
films the process fails.

20 According to this invention we have found a  
process which can be easily operated, even  
mechanically, for producing 3-color pictures,  
wherein the intermediate filter layers which are  
incapable of being removed by developing and  
fixing baths are retained unchanged until, ac-  
25 cording to the arrangement of the photographic  
layers one or two of the part-pictures have been  
converted into a colored picture, that is to say,  
when the filter layers are used not only for color  
separation in the exposure or copying operation  
30 (first exposure), but also for the purpose of con-  
verting the developed and fixed silver picture,  
converted into silver halide, into a colored pic-  
ture for the single exposure (second exposure)  
35 of the silver halide part-picture.

The process may be as follows:

A tri-pack material ready for exposure is made  
up in the following order:

- 40 1=blue sensitive layer
- 2=yellow filter
- 3=green sensitive layer
- 4=red filter
- 5=red sensitive layer.

45 The emulsions and filter layers are made by the  
usual methods. The yellow filter may, for ex-  
ample, be a gelatin layer which contains Fuller's  
yellow (Schultz Farbstofftabellen, 7th edition,  
Vol. I, No. 230; Vol. II, page 227) made insoluble  
50 by calcium nitrate, while the red filter layer may  
contain the aluminium lake of the dyestuff from  
diazotized naphthylamine and 2-hydroxy-naph-  
thalene-3,6-disulfonic acid.

55 After the exposure the material is developed  
and fixed in the usual manner whereupon the

silver pictures in the layers 1, 3 and 5 are con-  
verted into silver halide in known manner.

Now the layer 1 is exposed to blue light, where-  
by the light penetrating into the layer 2 will be  
completely absorbed, and is developed with a 5  
developer which yields a yellow picture, for ex-  
ample, a developer consisting of a solution of 5  
grams of 1-p-chlorophenyl-3-methyl-4-aminopy-  
razolone, 5 grams of dry sodium sulfite and 0.5  
gram of potassium bromide in 1000 cc. of water. 10  
Then layer 5 is exposed from the back of the film  
to blue light and developed blue-green (for ex-  
ample with dimethyl-para-phenylene-diamine  
and trichloronaphthol). In further baths the  
filter layers are now removed, for instance by 15  
means of a solution of sodium hydrosulfite or  
Rongalite (Schultz Farbstofftabellen, 7th edition,  
Vol. II, pages 295 and 296), and the silver pictures  
in 1 and 5 are dissolved in known manner. The  
filter layers are now removed, for instance by 20  
means of a solution of sodium hydrosulfite or  
Rongalite (Schultz Farbstofftabellen, 7th edition, Vol. I,  
No. 853), or toning process, for instance, by con-  
version into a picture being formed by nickel- 25  
dimethylglyoxime, or developed, after exposure,  
by a developer which yields a red picture (for  
example thioindoxyl). After fixation or separa-  
tion of the silver produced in the middle layer,  
the film contains three superimposed color-pic- 30  
tures which together give a complementary col-  
ored negative. From this any number of cor-  
rectly colored positives may be made by the same  
procedure. Instead of a color forming developer  
there may also be used a developer containing a 35  
color forming component.

The foregoing example deals only with one of  
the possible methods of applying the invention.  
The arrangement of the layers may, for example,  
be otherwise selected; for instance, one layer 40  
may be arranged on the back of the film. In  
this case the removal of the filter may follow the  
finishing of the first part-color picture if the  
production of the second and the third picture  
(rear side) picture is such that only one side of 45  
the film comes into contact with the baths.

What we claim is:

- 1. A photographic material which comprises a support, a photographic silver halide emulsion layer applied to said support, a filter layer con- 50  
taining as a red dye the aluminium lake of the  
dyestuff from diazotized naphthylamine and 2-  
hydroxy-naphthalene-3,6-disulfonic acid applied  
to said silver halide emulsion layer, a second  
silver halide emulsion layer applied to said red 55

- filter layer, a yellow filter layer dyed with Fuller's yellow made insoluble by calcium nitrate applied to said silver halide emulsion layer and a third silver halide emulsion layer applied to said yellow filter layer, the dyes of said red filter layer and said yellow filter layer being stable against treatment in the photographic treating baths and being decolorizable by one of the group consisting of sodium hydrosulfite and Rongalite.
- 5 2. A photographic material which comprises a support, a red-sensitive silver halide emulsion layer applied to said support, a filter layer containing as a red dye the aluminium lake of the dyestuff from diazotized naphthylamine and 2-hydroxy-naphthalene-3,6-disulfonic acid applied to said silver halide emulsion layer, a green-sensitive silver halide emulsion layer applied to said red filter layer, a yellow filter layer dyed with Fuller's yellow made insoluble by calcium nitrate applied to said silver halide emulsion layer and a blue-sensitive silver halide emulsion layer applied to said yellow filter layer, the dyes of said red filter layer and said yellow filter layer being stable against treatment in the photographic treating baths and being decolorizable by one of the group consisting of sodium hydrosulfite and Rongalite.
- 10 JOHN EGGERT.  
BRUNO WENDT.